

Feb. 16, 1926.

1,573,013

W. A. OGG

PROCESS OF SMELTING ORES OF VOLATILE METALS

Filed Feb. 7, 1925

2 Sheets-Sheet 1



Feb. 16, 1926.

1,573,013

W. A. OGG

PROCESS OF SMELTING ORES OF VOLATILE METALS

Filed Feb. 7, 1925

2 Sheets-Sheet 2

Fig. 2.



Inventor:  
William A. Ogg  
By Henry Booth Jauney & Farmer  
Atts.

## UNITED STATES PATENT OFFICE.

WILLIAM A. OGG, OF NEWTON, MASSACHUSETTS.

## PROCESS OF SMELTING ORES OF VOLATILE METALS.

Application filed February 7, 1925. Serial No. 7,561.

*To all whom it may concern:*

Be it known that I, WILLIAM A. OGG, a citizen of the United States, and a resident of Newton, county of Middlesex, State of Massachusetts, have invented an Improvement in Processes of Smelting Ores of Volatile Metals, of which the following description, in connection with the accompanying drawings, is a specification, like characters on the drawings representing like parts.

My invention relates to the smelting of material bearing volatilizable metals, particularly but not exclusively natural or concentrated ores of zinc, and has among its objects the accomplishment of an increased recovery of the metal values at low cost by an improvement in that process of smelting practiced with retorts and condensers. My improved method, which may be so practiced as to increase the ore treating capacity of a given furnace, securing a higher percentage recovery of the metal values, an increased yield of spelter per retort, and in addition to produce directly from the zinc bearing ore products of high economic value hitherto produced only by more costly processes involving the treatment of metallic zinc, will be best understood from the following description when read in light of the accompanying drawings showing one form of apparatus for practicing my invention, while the scope of my invention will be more particularly pointed out in the appended claims.

In the drawing:—

Fig. 1 shows more or less diagrammatically an arrangement of apparatus for practicing my invention; and

Fig. 2 is a section on the line 2—2 of Fig. 1.

The furnace commonly used for the reduction of zinc ores or ores of like volatilizable metals includes tiers of cylindrical retorts commonly made of fire clay or other suitable refractory material, which retorts are removably supported in the combustion chamber of the furnace. The ore which may be natural oxides, or sulphides converted to oxides by roasting, is mixed with reduction fuel, usually coal or coke free as far as pos-

sible from sulphur, and the mixture charged into the retort. In practice when smelting zinc bearing ores the retorts are subjected to a temperature of about 1300 degrees centigrade, which reduces the ore and being above the boiling point of zinc volatilizes the metal which passes out of the retort in the form of a vapor and is condensed to a liquid in a condenser, the latter consisting of a short frustoconical continuation of the retort projecting from the combustion chamber and being commonly detachably connected with the retort.

In practicing the smelting process now commonly employed with existing apparatus the regulation of the amount of retort charge and temperature is a matter of great nicety. The limitations of the material used for making the condensers, initial cost, and handling charges make it impractical to increase the cooling surface of the condenser above that of the condenser now commonly employed. The limitation to the use of a condenser with a relatively small cooling surface therefore makes it necessary in practice to limit the charge in the retort to a value which will produce a rate of vapor discharge into the condenser not in excess of the capacity of the condenser efficiently to liquefy the metal. This charge is materially below the full cubical capacity of the retort and consequently the limitations placed on the practice of the process by the condenser reduce the output of the furnace, and in addition make it necessary closely to regulate the temperature to reduce to a minimum the losses due to escaping vapors from the mouth of the condenser. With existing apparatus the metallurgist is confronted with two alternatives, that of running with the condensers too cold with consequent production of a high percentage of blue powder which will have to be redistilled with further losses, or that of running with the condensers too hot with consequent loss of vapor from the mouth of the condenser.

By way of an example of good practice with the prior method the retort is loaded with mixed ore and fuel to roughly 75 percent of its cubical capacity. The recovery of metal content is about 89.5 percent in

the form of spelter, and of the remainder about 7.75 percent is in the residue, about 1 percent is absorbed by the walls of the retort and condenser, and the remaining loss of 1.75 percent is principally in the form of escaping vapors from the mouth of the condenser which it is uneconomical to attempt to recover. The recovery of 32 pounds per twenty-four hour day of metal value in the form of spelter may be considered the maximum capacity of the condenser in its normal operation with the prior method.

Because of the increasing prices of coal and labor and increasing overhead charges necessary to the performance of the prior method the expense of producing the product has increased greatly and one object of the present invention is both to permit more ore to be treated at one time and to increase the percent recovery of metal values, thus minimizing the expense per unit of commercially available metal produced.

In accordance with the invention the retort is deliberately substantially overcharged beyond the capacity of the condenser to condense efficiently, and as a purpose of the invention is to secure a large recovery of spelter the condenser is operated at full condensing capacity for the given operating conditions. Sufficient heat is applied to the retorts substantially to reduce all the metal which is in oxidized form and a substantial fraction of the metal values is intentionally caused to escape from the condenser and is recovered by other means. By this deliberate overcharging of the retort so that a substantial percentage of the metal values vaporized is passed out from the condenser an increased recovery of spelter per retort is obtained, while the remaining metal values as will be pointed out later are collected as highly valuable products.

Referring to the drawing I have shown a furnace 1 of the regenerative type in which are formed gas passages 3 connected by means of suitable flues 5 and ports 7 to combustion chambers 9. In the combustion chambers are arranged tiers of retorts 11 each of which is provided with a condenser 13 projecting beyond the front of the furnace. The furnace described is of a common type and per se forms no part of my invention.

In practicing my invention I attach to the front of the furnace opposite the condensers suitable hoods 15 which may be supported in any suitable manner as for example by providing them with the flanges 17 fitting a channel 19 carried by the front of the furnace. Each hood is provided with observation holes 21 which may be provided with dampers 22 for regulating the amounts of air admitted.

Each hood is connected by means of a

pipe 23 having a gate valve 25 to a main suction pipe 27 leading to an exhaust fan or blower 29 so that the vapors escaping from the condensers may be conveyed from the furnace to suitable collecting means for the vapors, and for this purpose I have shown the discharge pipe 31 of the fan leading to cooling chambers 33 discharging into a bag house 35 in which are suspended cloth bags 37 releasably closed at their lower ends by any suitable means 39, as for example a cord.

Conveniently the vapors escaping from the condensers are burned in the hood to provide zinc oxide, and as the vapors are burned in a relatively cool atmosphere due to the excess of air, the zinc oxide is suddenly chilled to produce a very fine powder easily handled by the conveying means and having in itself a high commercial value.

Preferably the condenser mouths are plugged with a mixture of screened anthracite dust with enough ore to give it body which provides a porous plug for the condenser mouths acting as a filter which frees the vapors from dust and other solid impurities and further acts to materially prevent the escape of heavy vapors such as the lead content of the ore.

In operation if the ore charged has an appreciable cadmium content the same largely may be segregated from the bulk of the zinc content discharged from the condensers due to the fact that the cadmium ore reduces at a lower temperature and consequently more rapidly than the zinc, which makes it possible first to pass off vapors rich in cadmium and then after it has been determined that the most active reduction of cadmium is completed to open the bottom of the bags in the bag house and shake them to recover a product rich in cadmium, or if desired this high cadmium bearing fume may be collected in a separate bag house or settling chamber. As the lead content of the ore after reduction is less volatile than the zinc practically all the lead is collected in the condensers resulting in the production of zinc oxide low in discoloring lead impurities, and if an ore low in cadmium be provided because of the substantial elimination of the lead content and the burning of the vapors in a large excess of air the zinc oxide, after a subsequent treatment if necessary to remove carbon, will be analogous or equal in quality to the zinc oxide produced by the so called French process consisting of burning metallic zinc.

It will be noted that my improved process avoids the previously mentioned alternative of running the condenser so cool compared to the rate of vapor flow from the retorts as to produce a substantial portion of the metal values as blue powder, and that as a consequence it is not necessary to use the same degree of care in carrying out my

method as with the prior method. At the same time the current of air induced by the exhaust fan is directed over the condensers which it is believed keeps them cool enough as compared to the increased rate of vapor flow to function to condense an increased amount of spelter per retort as compared with the prior process.

As an example of my improved method 10 without limitation thereto I have found that a retort furnace having 405 retorts, using 280 retorts for roasted ore and 125 retorts for blue powder and other zinc bearing material collected as return products from the 15 next preceding smelting operation, will produce an average of 39.9 pounds of spelter per retort. In this example the retorts containing ore were charged on the average with 98.2 pounds of roasted ore mixed with 20 30 pounds of reduction fuel consisting of approximately 5 pounds of anthracite coal and 25 pounds of coke breeze, the zinc content of the roasted ore averaging 69.4 pounds per retort. If the return products 25 resulting from the smelting operation given as an example are assumed to be equal in metal value to the return products charged from the next preceding operation, which assumption I have found to be approximated 30 in practice, then the total production of metal values represents the recovery from the ore charged, which means that the spelter recovery averaged 57.7 pounds for each retort charged with ore. This spelter 35 recovery represents 83.1 percent of the metal values charged in the form of ore, and at the same time there was recovered in the bag house a product representing 3.1 pounds of zinc per retort of the total 405 retorts or 40 4.5 pounds per retort charged with ore, representing 6.5 percent of the metal values of the ore charged. The total recovery of metal values of the ore in this example of my method, which example is the average of 45 six operations, is .92 percent, which figure includes 2.4 percent in the form of zinc recovered from the condensers by jigging and not returned to the furnace.

As an example of the prior method I have 50 found on the same basis of computation as in the example given above, that with the same retorts and furnace, a retort charged with 75 pounds of roasted ore of the same composition having a metal content of 52.2 pounds mixed with 28 pounds of the same kind of reduction fuel produced 46.7 pounds of spelter, the latter representing 89.5 percent of the metal values of the ore charged. Thus it will be noted that not only does my 55 improved process increase the furnace output but it also secures an increased recovery of the metal values with a smaller ratio of reduction fuel to the roasted ore charged, all of which will be apparent from an inspection of the following table summarizing

the results of the above examples of my improved method and the prior method.

|                                                       | Improved method. | Prior method. | 70 |
|-------------------------------------------------------|------------------|---------------|----|
| Number of retorts charged with ore                    | 280              | 280           |    |
| Number of retorts charged with return products        | 125              | 125           |    |
| Ore charged per retort charged with ore               | 98.2#            | 75#           |    |
| Fuel charge per retort charged with ore               | 30#              | 28#           |    |
| Metal value of ore per retort charged with ore        | 69.4#            | 52.2#         | 75 |
| Spelter recovery from ore per retort charged with ore | 57.7#            | 46.7#         |    |
| Percent metal recovery from ore in bag house          | 6.5              | None          |    |
| Total percent recovery of metal values of ore charged | .92              | 89.5          |    |

80 In the above example of my improved method the retorts used each had on the average a total volumetric capacity of 1.41 cubic feet, and the charge per cubic foot of this total retort capacity amounted to 69.7 pounds of ore mixed with 21.3 pounds of reduction fuel, representing a utilization of about 98 percent of the total volumetric capacity of the retort. I have found that my invention can be efficiently practiced by 85 charging the retorts with ore and reduction fuel to their full cubical capacity, in which case the output of fume and spelter will be correspondingly increased without it being necessary materially to increase the reduction temperature. Conveniently this may be done by briquetting the ore and fuel, in which case a mixture of ore and reduction fuel mixed with a suitable binder will be 90 formed into briquettes under pressure, thus increasing the amount of metal values that may be charged into a retort of given capacity. As suitable for this purpose I may use a mixture of 70 percent of roasted ore, 95 5 percent of anthracite coal, 20 percent of coke breeze, and 5 percent of pitch, which mixture can be briquetted in any suitable briquette making machine.

The amount of zinc oxide produced by my method can be varied by varying either the 100 charge or temperature or both, but preferably by varying the charge. In the above example of my method the temperature was raised gradually from about 1000 degrees centigrade, at which temperature the reduction process will begin, to a maximum of 1450 degrees centigrade, reaching the latter temperature after the operation had continued for about 14 hours, and was maintained at that maximum temperature for about 5 105 hours, or until the operation was completed. By reducing this maximum temperature or the charge the production of zinc oxide would be decreased, and I have found that as a practical economic procedure a recovery 110 of about 2.5 percent of the metal values of the ore in the form of oxide is the minimum.

I am aware that it has been proposed to 115 collect the escaping vapors from a retort 120

furnace, but the proposed process has been merely one of gleanings the relatively slight losses resulting from the presence of vapors escaping from the condenser, which losses are necessarily low as heretofore explained, and the proposed process is not practical as the cost would be greater than the returns. With my improved method, on the contrary, I propose deliberately to overcharge the retorts as compared to the condenser capacity and to collect an economically material proportion of the metal charged to the retort after it has passed through the condenser as a substantial and intentional factor in the process. At the same time spelter recovery is an important object and the condensers are operated under such conditions as will secure a maximum production of that product.

20 While the process as described has some aspects of fractional distillation, especially in the selective recovery of lead and cadmium if present, it is primarily a smelting process of treating ore or other crude zinc bearing material with reduction fuel.

An important feature of the invention is the possibility of production in substantial quantity of a high grade zinc oxide although in a sense as a by-product of spelter production, and it will be observed that in absence of a market for the zinc oxide the same may be charged to the retorts as a concentrated product rich in zinc.

The invention is applicable to existing installations of retort furnaces and is exceedingly simple, requiring only a moderate installation charge for alteration of the usual existing plant arranged for carrying out the prior method of spelter recovery. As 40 a larger amount of ore may be treated in each retort at one time, an economy of expensive heating fuel per amount of ore treated is realized for it will be observed that furnace heat losses are substantially 45 independent of the amount of ore charged. Also as a greater amount of ore is heated at one time the overhead and labor charges are correspondingly reduced. The maximum effective production of metallic spelter is 50 provided for, yet a considerable fraction of the metal values is recovered exteriorly of the condenser.

Although I have described for purposes of illustration one specific manner of carrying out my improved method it is to be understood that I am not limited thereby to its particular details as described, but that within the scope of my invention wide deviations may be made therefrom without departing from the spirit of my invention.

Claims—

1. That method of smelting crude zinc bearing material utilizing a retort furnace and condenser, which consists in charging the retort with a mixture of said material

and reduction fuel in amount to produce a volume of metal vapors in substantial excess of the capacity of the condenser fully to condense the same and conducting the vapors discharged from the condenser, which comprise a considerable fraction of the metal values in the material treated, for recovery by deposit of the metal values therein while obtaining a recovery of spelter in the condenser to the full capacity thereof.

2. That method of smelting crude zinc bearing material utilizing a retort furnace and condenser, which consists in charging the retort with a mixture of said material and reduction fuel in amount to produce a volume of metal vapors in substantial excess of the capacity of the condenser fully to condense the same and conducting the vapors discharged from the condenser, which comprise a considerable fraction of the metal values in the material treated by a current of air, for recovery by deposit of the metal values therein while obtaining a recovery of spelter in the condenser to the full capacity thereof.

3. That method of smelting crude zinc bearing material utilizing a retort furnace and condenser, which consists in charging the retort with a mixture of said material and reduction fuel in amount to produce a volume of metal vapors in substantial excess of the capacity of the condenser fully to condense the same and conducting the vapors discharged from the condenser, which comprise a considerable fraction of the metal values in the material treated by a current of air directed against the condenser, for recovery by deposit of the metal values therein while obtaining a recovery of spelter in the condenser to the full capacity thereof.

4. That method of smelting crude zinc bearing material utilizing a retort furnace and condenser, which consists in charging the retort with a mixture of said material and reduction fuel in amount to produce a volume of metal vapors in substantial excess of the capacity of the condenser fully to condense the same and burning in an excess of air the vapors discharged from the condenser, which vapors comprise a considerable fraction of the metal values in the material treated, to produce a finely divided oxide while obtaining a recovery of spelter in the condenser to the full capacity thereof.

5. That method of smelting crude zinc bearing material utilizing a retort furnace and condenser, which consists in charging the retort with a mixture of said material and reduction fuel in amount to produce a volume of metal vapors in substantial excess of the capacity of the condenser fully to condense the same and burning in an excess of air the vapors discharged from the condenser, which vapors comprise a considerable fraction of the metal values in the

- material treated, to produce a finely divided oxide while obtaining a recovery of spelter in the condenser to the full capacity thereof and conducting the oxide by a current of air for recovery therefrom by deposit. 6. That method of smelting crude zinc bearing material utilizing a retort furnace and condenser, which consists in charging the retort with a mixture of said material and reduction fuel in amount to produce a volume of metal vapors in substantial excess of the capacity of the condenser fully to condense the same, directing a current of air against the condenser to increase the spelter-producing capacity thereof, burning in said current of air the vapors discharged from the condenser, which comprise a considerable fraction of the metal values in the material treated to produce a finely divided oxide and conducting the oxide by said current of air for recovery therefrom by deposit. 7. That method of smelting zinc bearing material utilizing a retort furnace and condenser, which consists in charging the retort with a mixture of said material and reduction fuel in substantial excess of the capacity of the condenser to condense fully the resulting metal vapors, burning the vapors discharged from the condenser in a current of air to produce a finely divided oxide, and collecting the oxide from said air by deposit in successive fractions to recover a fraction high in cadmium and a second fraction lower in cadmium while recovering spelter in the condenser to the full capacity thereof with condensation therein of substantially all the lead content of the material. 8. That method of smelting zinc bearing material utilizing a retort furnace and condenser, which consists in charging the retort with a mixture of said material and reduction fuel sufficient in amount to cause at least 2.5 percent of the metal values to be discharged in the form of vapor from the condenser mouth, and entraining said vapor by an air current flowing past the condenser mouth for recovery from said air by deposit. 9. That method of smelting zinc bearing material utilizing a retort furnace and condenser, which consists in charging the retort with a mixture of said material and reduction fuel sufficient in amount to cause at least 2.5 percent of the metal values to be discharged in the form of vapor from the condenser mouth, burning said vapor to produce an oxide, and entraining said oxide in a current of air for recovery from said air by deposit. 10. That method of smelting zinc bearing material utilizing a retort furnace and condenser, which consists in charging the retort with a mixture of said material and reduction fuel sufficient in amount to cause at least 2.5 percent of the metal values to be discharged in the form of vapor from the condenser mouth, directing a current of air against the condenser to increase its spelter producing capacity, burning the vapor in said air to produce a finely divided oxide, entraining said oxide in said air, and recovering said oxide from said air by deposit. 11. That method of smelting zinc bearing material utilizing a retort furnace and condenser, which consists in charging the retort to substantially its full cubical capacity with a mixture of said material and reduction fuel sufficient effectively to reduce the metal values and to produce a volume of metal vapors in substantial excess of the capacity of the condenser fully to condense the same, burning in air the vapors discharged from the condenser mouth, which comprise a considerable fraction of the metal values in the material treated, entraining the resulting oxides in a current of air, and recovering the oxides from said current of air by deposit. 12. That method of smelting zinc bearing material utilizing a retort furnace and condenser, which consists in charging the retort to substantially its full cubical capacity with a mixture of said material and reduction fuel sufficient effectively to reduce the metal values and to produce a volume of metal vapors in substantial excess of the capacity of the condenser fully to condense the same, directing a current of air against the condenser to increase the spelter producing capacity of said condenser, burning the vapors discharged from the condenser mouth in a current of air, and recovering the resulting oxides from said air by deposit. 13. That method of smelting zinc bearing material utilizing a retort furnace and condenser, which consists in charging the retort with a mixture of said material and reduction fuel in substantial excess of the capacity of the condenser to condense fully the resulting metal vapors, converting the vapors discharged from the condenser mouth and which comprise a considerable fraction of the metal values treated to a pulverulent solid compound by treating them with a gaseous substance which will combine with them, entraining said compound in a current of air, and separating the compound from said air by deposit. 14. That method of smelting zinc bearing material utilizing a retort furnace and condenser, which consists in charging the retort with a mixture of said material and reduction fuel in substantial excess of the capacity of the condenser to condense fully the resulting metal vapors, converting the vapors discharged from the condenser mouth and which comprise a considerable

fraction of the metal values treated to a 55  
pulverulent solid compound by treating  
them with a gaseous substance which will  
combine with them, entraining said com-  
pound in a current of air directed against  
said condenser for increasing its spelter pro-  
ducing capacity, and separating the com-  
pound from said air by deposit.

15. That method of smelting zinc bearing  
10 material utilizing a retort furnace and  
condenser, which consists in charging the  
retort to substantially its full cubical capacity  
with a mixture consisting of reduction  
fuel and a relatively large proportion  
15 of said material, heating the retort by pro-  
gressively raising the temperature to a  
maximum, maintaining said temperature at  
substantially said maximum until the reduc-  
tion is substantially completed to pro-  
20 duce during the reduction step a volume of  
metal vapors in substantial excess of the  
capacity of the condenser fully to condense  
the same, burning in an excess of air the  
vapors discharged from the condensers, com-  
25 prising a considerable fraction of the metal  
values treated, and recovering the metal  
values from the air by deposit.

16. That method of smelting zinc bearing  
30 material utilizing a retort furnace and  
condenser, which consists in charging the  
retort to substantially its full cubical capacity  
with a mixture of said material and reduction  
fuel, heating the retort by pro-  
35 gressively raising the temperature to a  
maximum, maintaining said temperature at  
substantially said maximum until the reduc-  
tion is substantially completed to produce  
during the reduction step a volume of metal  
40 vapors in substantial excess of the capacity  
of the condenser fully to condense the same,  
burning in an excess of air the vapors dis-  
charged from the condensers, comprising a  
considerable fraction of the metal values  
45 treated, and recovering the metal values  
from the air by deposit.

17. That method of smelting zinc bearing  
50 material utilizing a retort furnace and con-  
denser, which consists in charging the re-  
tort to substantially its full cubical capacity  
with a mixture of said material and reduction  
fuel, heating the retort by slowly rais-  
55 ing the temperature to a maximum, main-  
taining said temperature at substantially  
said maximum until the reduction is sub-  
stantially completed to produce during the  
reduction step a volume of metal vapors in  
60 substantial excess of the capacity of the  
condenser fully to condense the same, burn-  
ing in an excess of air the vapors dis-  
charged from the condensers, comprising a  
considerable fraction of the metal values  
65 treated, and recovering the metal values  
from the air by deposit.

18. That method of smelting zinc bearing

material utilizing a retort furnace and con- 65  
denser, which consists in charging the re-  
tort to substantially its full cubical capacity  
with a mixture of reduction fuel and said  
material, heating the retort by starting at  
substantially the temperature at which re- 70  
duction will begin, progressively raising  
this temperature to a maximum materially  
in excess of the starting temperature and  
maintaining said temperature at substan-  
tially said maximum until the reduction is 75  
substantially completed to produce during  
the reduction step a volume of metal vapors  
in substantial excess of the capacity of the  
condenser fully to condense the same, burn-  
ing in an excess of air the vapors discharged 80  
from the condenser mouths, comprising a  
considerable fraction of the metal values  
treated, and recovering the metal values  
from said air by deposit.

19. That method of smelting zinc bearing  
85 material utilizing a retort furnace and con-  
denser, which consists in compressing a  
mixture of said material and reduction fuel,  
charging the retort with the compressed  
mixture in amount to produce a rate of 90  
vapor flow in excess of the capacity of the  
condenser efficiently to condense said vapor,  
burning in an excess of air the vapor dis-  
charged from the condenser mouth, com-  
prising a considerable fraction of the metal 95  
values treated, and recovering the metal  
values from said air by deposit.

20. That method of smelting zinc bearing  
100 material utilizing a retort furnace and con-  
denser, which consists in compressing a  
mixture of said material and reduction fuel,  
charging the retort with the compressed  
mixture to substantially the full cubical 105  
capacity of said retort to produce a rate  
of flow of metal vapor in substantial excess  
of the capacity of the condenser fully to  
condense the same, burning in an excess of  
air the vapor discharged from the con- 110  
denser mouth, comprising a considerable  
fraction of the metal values treated, and re-  
covering the metal values from said air by  
deposit.

21. That method of smelting zinc bearing  
115 material utilizing a retort furnace and con-  
denser, which consists in briquetting a  
mixture of said material and reduction fuel,  
charging the retorts with the briquettes in  
amount to produce a rate of vapor flow in  
120 substantial excess of the capacity of the  
condenser efficiently to condense said vapor,  
burning in an excess of air the vapor dis-  
charged from the condenser mouth com-  
prising a considerable fraction of the metal  
125 values treated, and recovering the metal  
values from said air by deposit.

22. That method of smelting zinc bearing  
material utilizing a retort furnace and con-  
denser, which consists in briquetting a mix-

ture of said material and reduction fuel, vapor discharge from the condenser mouth, charging the retorts with the briquettes to comprising a considerable fraction of the substantially the full cubical capacity of metal values treated, and recovering the 10 said retort to produce a rate of flow of metal values from said air by deposit. In testimony whereof, I have signed my metal vapor in substantial excess of the capacity of the condenser fully to condense the same, burning in an excess of air the

WILLIAM A. OGG.